# EUROPEAN PATENT SPECIFICATION

(11) **EP 0 577 124 B1**
(45) Date of publication and mention of the grant of the patent: **16.10.2002**
(21) Application number: 93110517.5
(22) Date of filing: 01.07.1993
(51) Int. Cl.: C21D 8/12

(54) **Grain oriented electrical steel sheet having high magnetic flux density and ultra low iron loss and process for producing the same**
Kornorientiertes Elektroblech mit hoher Flussdichte und geringen Eisenverlusten und Herstellungsverfahren
Tôle d'acier électrique à grains orientés ayant une haute densité de flux et une faible perte dans le fer et procédé d'élaboration

(30) Priority: 02.07.1992 JP 17579092; 03.08.1992 JP 20679592; 19.08.1992 JP 22050092; 22.10.1992 JP 28478792; 12.11.1992 JP 30272892; 21.12.1992 JP 34074692
(43) Date of publication of application: 05.01.1994
(73) Proprietor: NIPPON STEEL CORPORATION, Tokyo 100-12 (JP)
(72) Inventor: Tanaka, Osamu, c/o Nippon Steel Corp. Yawata, Kitakyushu-shi, Fukuoka (JP); Kuroki, Katsuro, c/o Nippon Steel Corp. Yawata, Kitakyushu-shi, Fukuoka (JP); Ishiba, Maremizu, c/o Nippon Steel Corp. Yawata, Kitakyushu-shi, Fukuoka (JP); Masui, Hiroaki, c/o Nippon Steel Corp. Yawata, Kitakyushu-shi, Fukuoka (JP); Haratani, Tsutomu, c/o Nippon Steel Corp. Yawata, Kitakyushu-shi, Fukuoka (JP); Nakamura, Yoshio, c/o Nippon Steel Corp. Yawata, Kitakyushu-shi, Fukuoka (JP); Honma, Hotaka, c/o Nippon Steel Corp. Yawata, Kitakyushu-shi, Fukuoka (JP); Mishima, Yoichi, c/o Nippon Steel Corp. Yawata, Kitakyushu-shi, Fukuoka (JP)
(74) Representative: VOSSIUS & PARTNER

(56) References cited:
- EP-A- 0 305 966
- EP-A- 0 392 534
- EP-A- 0 420 238
- EP-A- 0 488 726
- EP-A- 0 525 467
- EP-A- 0 565 029
- EP-A- 0 566 986
- FR-A- 2 445 377
- GB-A- 1 480 514
- JP-A- 60 131 976
- US-A- 3 671 337
- US-A- 3 856 568
- US-A- 4 032 366
- US-A- 4 367 100
- US-A- 4 543 134
- DATABASE WPI Section Ch, Week 7815, Derwent Publications Ltd., London, GB; Class M27, AN 78-27745A & JP-A-53 022 113 (KAWASAKI STEEL) 1 March 1978
- PATENT ABSTRACTS OF JAPAN vol. 8, no. 212 (C-244) 27 September 1984 & JP-A-59 096 278 (KAWASAKI SEITETSU) 2 June 1984
- PATENT ABSTRACTS OF JAPAN vol. 3, no. 142 (C-65) 24 November 1979 & JP-A-54 120 215 (SHIN NIPPON SEITETSU) 18 September 1979

## Description

The present invention relates to a grain oriented electrical steel sheet not having a glass film (a forsterite film) and particularly to a grain oriented electrical steel sheet having a high magnetic flux density and an ultra low iron loss and remarkably excellent workability, such as slittability, cuttability and punchability, and a process for producing the same.

Grain oriented electrical steel sheets are used mainly as an iron core material for transformers and other electrical equipment and should be excellent in magnetic properties, such as inductions and an iron loss property.

In order to obtain good magnetic properties, it is necessary to highly arrange the <001> axis which is an easily magnetizable axis in the direction of rolling. Further, sheet thickness, grain size, specific resistance, film, etc. are also important because they have a great influence on the magnetic properties.

The orientation of grains has been remarkably improved by a method characterized by a high reduction ratio in final cold rolling wherein AlN and MnS are used as an inhibitor, so that, at the present time, it has become possible to provide steel sheets having a magnetic flux density close to the theoretical value. On the other hand, film properties and workability in addition to magnetic properties are important to the use of grain oriented electrical steel sheets by customers. In general, grain oriented electrical steel sheets are treated with a film having a double layer structure comprising a glass film formed in the final box annealing and an insulating film. The glass film is composed mainly of forsterite (Mg₂SiO₄) that is a product of a reaction of MgO as an annealing separator with SiO₂ formed during decarburization annealing. This ceramic film is hard and highly resistant to abrasion and has a significant adverse effect on durability of tools used in working of electrical steel sheets, such as slitting, cutting and punching. For example, when grain oriented electrical steel sheets having a glass film are subjected to punching, there occurs abrasion of molds and the occurrence of burr in the sheet at the time of punching becomes significant after effecting the punching about several thousand times, which leads to problems of use. For this reason, it becomes necessary to effect regrinding of molds or replacement of the molds with new molds. This lowers the working efficiency in the working of iron cores by customers and incurs an increase in the cost. With respect to the magnetic properties of the electrical steel sheets, although an improvement in the iron loss can be certainly attained by virtue of the tension of the film, in some forming conditions an increase in the thickness of the film or other unfavorable phenomenon unfavorably gives rise to a lowering in the magnetic flux density due to the presence of non-magnetic substances. For this reason, in the case of thick materials wherein improvement of the iron loss by the tension of the film is expected, or in the case where the iron loss can be improved by the division of the magnetic domain using other means, grain oriented electrical steel sheets not having a glass film are desired rather than grain oriented electrical steel sheets having a glass film because of the above-described problem.

Especially, in recent years, techniques using optical, mechanical and chemical means have been developed for refining the magnetic domain, which enables the iron loss to be improved without the tension of the glass film, and it has become apparent that the grain oriented electrical steels sheet not having a glass film are advantageous over those having a glass film by virtue of the absence of an adverse effect of an internal oxide layer of the glass film which causes a pinning phenomenon with respect to the movement of the domain wall in the magnetization. For this reason, there is an ever-increasing demand for the development of a grain oriented electrical steel sheet having a high magnetic flux density and not having a glass film which is important when various working conditions used by customers are taken into consideration.

A process for producing a grain oriented electrical steel sheet not having a glass film is disclosed, for example, in JP-A-53-22113. In this process, the thickness of an oxide film is brought to 3 µm or less in the decarburization annealing, particular alumina containing 5 to 40% of a hydrous silicate mineral powder is used as an annealing separator, and final annealing is effected with this annealing separator coated on the steel sheet. According to the description of the specification, this method reduces the thickness of the oxide film, enables an easily removable glass film to be formed by virtue of the incorporation of the hydrous silicate mineral and provides a steel sheet having a metallic gloss. As a method for inhibiting the formation of a glass film by using an annealing separator, JP-A-56-65983 discloses a technique wherein an annealing separator comprising aluminum hydroxide and, incorporated therein, 20 parts by weight of an additive for removing impurities and 10 parts by weight of an inhibitor is coated on a steel sheet to form a thin glass film having a thickness of 0.5 µm or less. Further, JP-A-59-96278 proposes an annealing separator comprising Al₂O₃, which is less reactive with SiO_{2,} as an oxide layer formed in the decarburization annealing and MgO which has an activity lowered by sintering at a high temperature of 1,300°C or above. According to the description of the specification, the proposed annealing separator can inhibit the formation of forsterite.

EP-A-0 305 966 discloses a method for producing glassless grain-oriented electrical steel sheet using no AlN as inhibitor and exhibiting metallic luster by applying an annealing separator consisting of magnesium blended with one or more salts of alkali metal or alkali or alkali-earth metal.

EP-A-0 420 238 discloses a process for preparing a grain-oriented steel sheet having high magnetic flux density, in which nitriding is performed and a glass coating is formed in the final products.

All the above-described prior art techniques are based on a low-quality grain oriented electrical steel sheet having a magnetic flux density as low as 1.88 Tesla or less usually called "orient core", and no technique for stably providing a grain oriented electrical steel sheet having a high magnetic flux density contemplated in the present invention has hitherto been developed in the art.

An object of the present invention is to provide a grain oriented electrical steel sheet having a high magnetic flux density and an ultra low iron loss, which grain oriented electrical steel sheet has excellent punchability, slittability, cuttability, etc. and substantially evenly free from a glass film, and a process for producing said steel sheet at a low cost on a commercial scale.

The most characteristic feature of the material according to the present invention resides in that the material is a grain oriented electrical steel sheet not having a glass film or having no significant glass film. This characteristic feature leads to two effects. One is that the workability, such as slittability, cuttability or punchability, is excellent. Since the glass film comprises a hard ceramic, it accelerates the abrasion of working tools and reduces the workability. The second effect is to reduce the iron loss after the refining of the magnetic domain. The iron loss is divided into a hysteresis loss as a dc component and an eddy current loss as an ac component. The eddy current loss can be decreased by reducing the sheet thickness. In this case, however, if a glass film is present on the surface of the steel sheet, since the interface of the matrix and the glass film is not smooth, the hysteresis loss increases, so that no satisfactory effect of reducing the iron loss can be attained and, rather, the iron loss increases. The feature of the mechanism for reducing the iron loss of the material according to the present invention is that the material has no glass film and has a smooth interface.

In general, the iron losses become lower with increasing B₈ value (i.e., magnetic flux density at a magnetizing force of 800 A/m). In the present invention, however, mere increase in the B₈ value does not result in a lowering of the iron loss. This is because an increase in the B₈ value gives rise to an increase in the width of the magnetic refining in turn increases the abnormal eddy current loss. This effect becomes significant with an increase in the smoothness of the surface of the steel sheet. For this reason, in order to sufficiently attain the effect of reducing the iron loss in the material according to the present invention, it is necessary to enhance the B₈ value and, at the same time, to use a technique for decarburization the magnetic domain. The formation of grooves, flaws or the like on the surface of the steel sheet by using means, such as a laser beam, a gear wheel, a press, a ball-point pen and etching, is useful for this purpose. Further, coating of a film capable of imparting a high tension while maintaining the smoothness of the surface of the steel sheet is also useful.

In the present invention, in order to produce a grain oriented electrical steel sheet of the type described above, use is made of the following specific steps. First, the amount of an oxide layer formed on the surface of the steel sheet after final box anealing is minimized. This is because the oxide layer derived from the decarburization annealing causes the occurrence of a reaction of magnesia, as an annealing separator, to form a glass film. Second, additives including Cl compounds are added to the annealing separator. These additives have a feature that they form a glass film during final box annealing and then remove the glass film. In order to provide a steel sheet having a high B₈ value, in the course of final box annealing involving the progress of the secondary recrystallization, precipitates called "inhibitor", which serves to regulate the grain boundary movement in the steel sheet, should be present in a limited amount under certain specific conditions and, after the secondary recrystallization, should disappear. The complicated behavior of the inhibitor is governed by the glass film. Therefore, also in the production of the material according to the present invention, although the glass film should be present for the progress of the secondary recrystallization, it should preferably disappear after the secondary recrystallization. On the other hand, for example, Cl compounds or the like generally have a melting point below the glass film formation temperature and accelerate the formation of a glass film during final box annealing. However, when the temperature is above the glass film formation temperature, the Cl contained in the compound etches the interface of the film and the matrix and removes the glass film.

A further method for enhancing the B₈ value is to increase the partial pressure of nitrogen in the finish-annealing atmosphere. This is the third characteristic feature of the present invention. In order to provide a grain oriented electrical steel sheet having a high B₈ value, the present invention is based on the assumption that nitrides are used as the inhibitor. However, weakening of the inhibitor attributable to denitriding is the greatest problem in the step of rendering the material glassless. Although the presence of a glass film in the course of the secondary recrystallization as described above in connection with the second characteristic feature is a measure for preventing denitriding, it is necessary to maintain the partial pressure of nitrogen in the final box annealing atmosphere at a certain value or higher for the purpose of further reinforcing this effect.

The invention will be described in connection with the drawings, in which:
Figs. 1A, 1B and 1C are diagrams for showing final box annealing conditions; and
Fig. 2 is a diagram showing the relationship between the primary grain diameter and the decarburization annealing temperature.

Basically, in the production the grain oriented electrical steel sheet having a high magnetic flux density and an ultra-low iron loss according to the present invention, inhibitor elements, for example, Al, N, Mn and S, are not completely dissolved in the steel at the stage of heating a slab, the material is nitrided in a strong reducing atmosphere after decarburization annealing to form an inhibitor composed mainly of (Al, Si)N, and a good secondary recrystallization is developed in final box annealing, followed by the division of the magnetic domain.

The process for producing the grain oriented electrical steel sheet having a high magnetic flux density and not having a glass film according to the present invention using a starting material having the above-described composition and the above-described steps is characterized by a series of treatments conducted between decarburization annealing and final box annealing.

The material subjected to cold rolling to a final sheet thickness is subjected to decarburization annealing in a continuous line. In the decarburization annealing, C in the steel is removed, and primary recrystallization is effected. At the same time, an oxide film composed mainly of SiO₂ is formed on the surface of the steel sheet. In this case, the degree of oxidation of the steel sheet is the first characteristic feature of the present invention, wherein the oxygen content is 900 ppm or less, and an Fe-oxides to SiO₂ ratio is 0.20 or less.

The decarburization annealing is effected at 800 to 875°C in an atmosphere comprising N₂ and H₂ while controlling the dew point. Subsequently, in the second half of the decarburization annealing or after the completion of the decarburization annealing or in both the above-described stages, a nitriding treatment is effected in the same line or a separately provided line. In this case, the optimal nitrogen content is 150 ppm or more, preferably 150 to 300 ppm although it depends upon the primary recrystallized grain diameter.

Thereafter, the material is coated with an annealing separator, dried, coiled and subjected to final box annealing. In this case, the composition of the annealing separator is the second characteristic feature of the present invention and plays an important role in the formation and regulation of a glass film and the decomposition reaction of the glass film. In the annealing separator used in the present invention, MgO has a particle size distribution such that 30% or more of the MgO consists of particles having a diameter of 10 µm or less. Further, it should have a CAA value of 50 to 300 sec and a hydrated water content of 5% or less. Further, a compound composed mainly of a Cl compound is used as an additive to the MgO. In the production of products not having a glass film, a smooth steel sheet surface and a good iron loss property, the Cl compound underlies the invention of the instant application in that it serves to remove the glass film formed during the final finish annealing. The glass film serves to regulate a nitriding reaction and a denitriding reaction during the final box annealing and to regulate the inhibitor content of the steel sheet. Therefore, mere formation of a glass film cannot provide the development of good secondary recrystallized grains, so that it is impossible to attain the iron losses reduction effect derived from a smooth steel sheet interface. For this reason, in order to provide a grain oriented electrical steel sheet having a high magnetic flux density and an ultra-low iron loss, which is the principal object of the present invention, it is necessary to form a glass film which is then removed. The Cl compound accelerates a reaction of SiO_{2,} formed on the surface of the steel sheet in the decarburization annealing, with MgO, as the annealing separator, to form a glass film at a lower temperature than that usually necessary for the formation of the glass film, and then forms a chloride of iron at the interface of the film and the matrix to remove the film. Besides the Cl compounds, S compounds, carbonates, nitrates and sulfates cause the above-described reaction, and Li, K, Bi, Na, Ba, Ca, Mg, Zn, Fe, Zr, Sn, Sr end Al are useful as an element combined therewith. In the process according to the present invention wherein secondary recrystallization is developed by the step of heating of a slab at a low temperature + nitriding after decarburization annealing, the Cl compound is most effective in attaining a high magnetic flux density.

With respect to the amount of addition of such a compound, when the amount is less than that specified in the claim, no satisfactory effect of removing the film can be attained, while when the amount is excessively large, the magnetic flux density falls. Thus, it becomes possible to provide a grain oriented electrical-steel sheet having no a glass film comprising forsterite and/or spinel or having no significant glass film.

Besides the annealing separator, the final box annealing conditions, as the third characteristic feature of the present invention, are important to the present invention.

Extensive experiments and studies conducted by the present inventors have revealed that annealing atmosphere conditions are an important factor for stabilizing the secondary recrystallization and increasing the magnetic flux density when, like the present invention, use is made of the step of effecting a nitriding treatment after decarburization annealing to form an inhibitor composed mainly of (Al, Si)N and regulating the formation of a glass film and causing a decomposition reaction of the glass film by using an annealing separator and final finish annealing conditions.

Specifically, when an (Al, Si)N inhibitor is utilized substantially without using a MnS as the inhibitor as in the present invention, the secondary recrystallization initiates at about 1,100°C which is higher than that in the case of the conventional process for producing a grain oriented electrical steel sheet having a high magnetic flux density. For this reason, it is necessary to maintain the strength of the inhibitor at a constant level while effecting the inhibition of formation of the glass film and the decomposition reaction of the glass film until the temperature reaches the secondary recrystallization initiation region.

The reason for this is that, in the process where the annealing separator once initiates the formation of a glass film and then induces the decomposition reaction of the glass film, the decomposition of the inhibition in the steel rapidly proceeds from the point in time when the decomposition reaction of the glass film begins. For this reason, neither good secondary recrystallization nor high magnetic flux density can be attained without effecting finish annealing under specific conditions according to the present invention.

With respect to final box annealing conditions, in the temperature rise during which the decomposition reaction of the glass film begins, the temperature is raised in an atmosphere having a N₂ content of 30% or more until it reaches the soaking temperature. This enables (Al, Si)N to be stabilized until the secondary recrystallization begins. The heating rate in the final box annealing is 20°C/hr or less. When it exceeds 20°C/hr, the growth rate of secondary recrystallization becomes improper, which deteriorates the integration density in the orientation of the product, so that a satisfactorily high B₈ value cannot be obtained.

The steel sheet subjected to final box annealing is then subjected to baking with an insulating coating solution and heat flattening combined with shape reforming and stress relieving annealing in a continuous annealing line at 800 to 900°C. Before or after the heat flattening, a seam or spotty recess having a depth of 5 to 50 µm is imported at intervals of 2 to 15 mm in a direction at an angle of 45 to 90° to the rolling direction by a laser beam, a sprocket roll, a press, marking, local etching, etc. Thereafter, various insulating coating solution are coated according to applications on the part of the customers, and the coated material is subjected to a baking treatment. When the insulating coating solution is used for the purpose of imparting film tension, the steel sheet is coated with a coating solution comprising a phosphate or colloidal silica as described in JP-B-53-28375 and then subjected to a baking treatment. Further, when a good workability is needed in the use thereof on the part of the customers, the surface of the steel sheet subjected to heat flattening is coated with an organic coating solution or a semi-organic coating solution and then subjected to a baking treatment. Alternatively, the surface of the steel sheet subjected to heat flattening may be coated with an inorganic coating solution, subjected to a baking treatment and then coated with an organic coating solution and subjected to a baking treatment to form a film having a double layer structure. When use is made of the organic film forming agent, (1) at least one totally organic coating solution selected from acrylic, polyvinyl, vinyl acetate, epoxy, styrene and other resins and/or their polymers and crosslinking products, or (2) a semi-organic coating solution comprising a mixture of the resin recited in the above item (1) with at least one member selected from chromates, phosphoric acid, phosphates, boric acid, borates, etc. is coated and baked at a temperature in the range of from 150 to 450°C to a thickness of 2 to 6 µm before use of the steel sheet.

The coating and baking treatment with these organic coating solution contributes to a remarkable improvement in the slittability, cuttability, punchability, etc. With respect to the punchability, the conventional products having a glass film can be punched about 5000 times when use is made of a steel die. On the other hand, according to the present invention, in products, wherein the thickness of the glass film is 0.3 µm or less, the punchability can be improved to about 100,000 times when an inorganic insulating coating solution agent is coated and baked, and to about 2,000,000 times when a semi-organic film forming agent is further coated and baked thereon.

The reason for the limitation of the constituent features of the present invention will now be described.

At the outset, the reason for the limitation of the chemical compositions of the electrical steel slab used as the starting material will be described.

With respect to the C content, when the content is less than 0.021%, the secondary recrystallization becomes so unstable that the magnetic flux density of the product is as low as about 1.80 Tesla in terms of the B₈ value even in the case of successful secondary recrystallization. On the other hand, when the C content exceeds 0.075%, the decarburization annealing time should be prolonged, so that the productivity is lowered.

With respect to the Si content, the specific resistance of the product varies depending upon the Si content. When the Si content is less than 2.5%, satisfactory iron loss value is not obtained. On the other hand, when it exceeds 4.5%, cracking and breaking of the material frequently occur during cold rolling, which makes it impossible to stably effect the cold rolling operation.

One of the characteristic features of the composition system of the starting material according to the present invention is to limit the S content to 0.014% or less. In the prior art, for example, in a technique disclosed in JP-B-47-25220, S (sulfur) is described as an element for forming as MnS a precipitate necessary for inducing secondary recrystallization, and there exists a content range capable of exhibiting the best effect, which content range has been specified as an amount range capable of dissolving, in a solid solution form, MnS at the stage of heating the slab prior to the hot rolling. As a result of studies in recent years, it has been found that S aggrarate the poor secondary recrystallization when a slab of a material having a high Si content is heated at a low temperature and hot-rolled in a process for producing a unidirectionally grain oriented electrical steel sheet where (Al, Si)N is used as a precipitate necessary for secondary recrystallization. When the Si content of the material is 4.5% or less, if the S content is 0.014% or less, preferably 0.0070% or less, poor secondary recrystallization does not occur at all.

In the present invention, use is made of (Al, Si)N as a precipitate necessary for the secondary recrystallization. In order to ensure the necessary minimum AlN, it is necessary for the acid-soluble Al content and N content to be 0.010% or more and 0.0030% or more, respectively. However, when the acid-soluble Al content exceeds 0.040%, the AlN content during hot rolling become improper, which renders the secondary recrystallization unstable. For this reason, the acid-soluble Al content is limited to 0.010 to 0.040%. On the other hand, when the N content exceeds 0.0130%, not only there occurs surface cracking called "blister" on the surface of the steel sheet but also the primary recrystallized grain diameter cannot be regulated. For this reason, the N content is limited to 0.0030 to 0.0130%.

When the Mn content is less than 0.05%, the secondary recrystallization becomes unstable. However, when it is excessively high, although the B₈ value becomes high, the use of Mn in an amount exceeding a certain value is disadvantageous from the viewpoint of cost. For this reason, the Mn content is limited to 0.05 to 0.45%.

The decarburization annealing according to the present invention should satisfy requirements that the oxygen content should be 900 ppm or less and the Fe-oxides to SiO₂ ratio is 0.20 or less. When the oxygen content exceeds 900 ppm, the SiO₂ and Fe-oxides contents inevitably increase and the thickness of the oxide film as well becomes large, which is disadvantageous for the glass film decomposition reaction in the final box annealing. Specifically, SiO₂ remains just under the surface, which weakens the effect of improving the workability or makes it impossible to bring the surface to a completely specular glassless state. Further, this is causative of the deterioration of the magnetic properties. Moreover, since the formation of excessive SiO₂ accelerates the decomposition of AlN etc. as the inhibitor in the steel by the action of SiO₂ prior to the initiation of the secondary recrystallization, there occurs a problem that a good orientation cannot be attained. However, when the degree of oxidation is extremely limited, the decarburization time should be prolonged, so that the productivity is lowered. The degree of oxidation is preferably in the range of from 400 to 700 ppm in terms of the oxygen content.

When the P content is 0.045% or less in the production of a steel by a melt process, the effect of enhancing the magnetic flux density is small. On the other hand, when the P content exceeds 0.20%, the sheets becomes so fragile that it becomes difficult to effect cold rolling.

The P content of the product is important to the present invention. P is dissolved in a solid solution form in iron, and part thereof is present in a precipitated state. The P is very useful for reducing the iron loss of the product, and in order to attain the effect, it is necessary for the P content to be 0.03% at the lowest. On the other hand, the P content exceeds 0.15%, the product becomes fragile, which is detrimental to the workability of the product, for example, punchability, so that the product is unsuitable for use.

The Fe-oxides to SiO₂ ratio in the oxide film is limited to 0.20 or less. When this ratio exceeds 0.20, since the glass film formation reaction is remarkably accelerated in the first half of the finish annealing, the amount of formation of the forsterite is increased, which inhibits the reaction in the subsequent step of decomposing the forsterite from sufficiently proceeding. When the FeO to SiO₂ ratio is 0.20 or less, it is possible to provide a steel sheet having substantially no glass film. after the completion of the finish annealing by virtue of effects attained, for example, by the addition of additives to MgO.

The nitrogen content of the steel sheet after the completion of the decarburization annealing is limited to 150 ppm or more. This requirement should be satisfied for the purpose of forming the inhibitor (Al, Si)N necessary for stably providing good secondary recrystallized grains in the process of the present invention. When the nitrogen content is less than 150 ppm, the secondary recrystallization becomes so unstable that fine grains are liable to occur. On the other hand, when the nitrogen content exceeds 300 ppm, roughness and unevenness occurs in the surface of the steel sheet in subsequent reactions, such as a denitriding reaction, or such a high nitrogen content often becomes disadvantageous in the step of purification after that. For this reason, it is desirable for the nitrogen content to be 300 ppm or less.

In MgO used in the annealing separator, there is a limitation on the particle diameter, CAA value and hydration ig-loss.

In the technique according to the present invention, the material is rendered glassless by decomposing and removing, through a chemical reaction, a moderate glass film formed in the first half of the temperature rise in the final box annealing. Specifically, in order to stabilize the inhibitor until the initiation of the secondary recrystallization in the first half of the final box annealing, it is necessary to utilize at this period the effect of preventing the additional oxidation, nitriding, etc. by a suitable amount of a glass film, and this is important to provide a glassless product having excellent magnetic properties.

For this purpose, it is important for the MgO as themain component of the annealing separator, as such, to have a suitable reactivity. Specifically, when the reactivity of MgO is very low, the reaction for the formation of the forsterite in the first half of the temperature rise in the final box annealing does not proceed, so that sealing effect cannot be attained by the film. In this case, even in the case of successful secondary recrystallization, the crystal orientation becomes very poor, or additional oxidation causes residual SiO₂, Al₂O₃ or their spinel to occur just under the surface of the steel sheet, which deteriorates the iron losses. For this reason, MgO is limited to have such a particle size distribution such that 30% or more of the MgO particles have a diameter of 10 µm or less. When this proportion is less than 30%, the reactivity becomes so low that the above-described effect cannot be attained. Further, the CAA value of MgO is limited to 50 to 300 sec. When this value is less than 50 sec, the progress of the hydration becomes very rapid for use on a commercial scale, so that it becomes difficult to control the hydration ig-loss. On the other hand, when the CAA value exceeds 300 sec, the reactivity of the MgO particles becomes so low that it becomes impossible to form a moderate forsterite in the first half of the final box annealing. The hydration ig-loss of MgO is limited to 5% or less. When the water content exceeds 5%, the dew point between steel sheets becomes so high that additional oxidation occurs in the first half of the temperature rise, which makes it difficult to render the surface of the steel sheet homogeneously glassless. In extreme cases, this has an influence even on the inhibitor, which aggravates the poor secondary recrystallization.

With respect to additives to MgO, at least one member selected from chlorides, carbonates, nitrates, sulfates and sulfides of Li, K, Bi, Na, Ba, Ca, Mg, Zn, Fe, Zr, Sn, Sr, Al, etc. is incorporated in an amount of 2 to 30 parts by weight based on 100 parts by weight of MgO. The addition of these compounds first causes a moderately thin forsterite film to be formed on the surface of the steel sheet in the first half of the temperature rise in the finish annealing. Then, the formation of the forsterite is inhibited, and additional oxidation is prevented. In the second half of the temperature rise, the film layer is decomposed by an Fe etching reaction in the film layer, thus rendering the surface of the steel sheet glassless. When the amount of addition of these compounds is less than 2 parts by weight, the decomposition reaction of the forsterite formed in the first half of the temperature rise does not sufficiently proceed, so that the glass film unfavorably remains unremoved. On the other hand, when the amount of addition of the above-described compounds exceeds 30 parts by weight, component elements in the additive unfavorably diffuse and penetrate into the steel sheet to give rise to intergranular etching or to have an influence on the inhibitor or on subsequent purification treatment. The amount of addition is particularly preferably in the range of from 5 to 15 parts by weight.

Final box annealing conditions are very important to the process according to the present invention wherein the formation of a moderate glass film and the decomposition of the glass film are effected in the final box annealing.

In general, N₂, H₂ or a mixed gas comprising N₂ and H₂ is used as the atmosphere gas in the final box annealing of grain oriented electrical steel sheets. The use of a mixed gas comprising N₂ and H₂ is advantageous from the viewpoint of the regulation of oxidation on the surface of the steel sheet and the cost. In the present invention, in order to regulate the strength of the inhibitor in the reaction for rendering the surface of the steel sheet glassless, an atmosphere having a N₂ content of at least 30% or more and comprising N₂, H₂ and another inert gases is used as an atmosphere gas during the temperature rise. When the partial pressure of N₂ is less than 30%, the effect of preventing the weakening of (Al, Si)N caused during the reaction for rendering the surface of the steel sheet glassless cannot be attained, so that a material having a high magnetic flux density cannot be stably provided. The deterioration of the magnetic properties is significant particularly under such an atmosphere condition that the N₂ content is 20% or less. When the atmosphere comprises 100% of N₂, in some property values, oxidation occurs due to an increase in the degree of oxidation between steel sheets, which often causes the surface of the steel sheet to become uneven. The N₂ content is preferably in the range of from 30 to 90%.

In the use of a gas having a N₂ content of 30% or more, although the steel sheet may be annealed in this atmosphere over the whole period of the temperature rise, additional oxidation may occur depending upon MgO conditions, so that it is preferred to change the atmosphere gas after the temperature reaches about 700°C which is most effective for stabilizing (Al, Si)N.

In the present invention, it is advantageous that the soaking temperature in the final box annealing is in the range of from 1180 to 1250°C. In the present invention, the material is in a glassless state at a point of time when the temperature has reached the soaking temperature in the final box annealing. The exposure of the material to the soaking temperature gives rise to further thermal etching, which renders the surface of the steel sheet specular. When the soaking temperature is below 1180°C, not only is this effect small but also the purification is disadvantaged. On the other hand, when the soaking temperature exceeds 1250°C, the effect of rendering the surface of the steel sheet specular is limited and there is a possibility that the form of the coil becomes poor and seizing occurs in the edge portion. The heating rate in the final box annealing is limited to 20°C/hr or less. When the heating rise rate exceeds this value, the decomposition rate of the inhibitor exceeds the growth rate of the secondary recrystallized grain, which inhibits the growth of crystal grains having an optimal orientation, so that the B₈ value falls.

Thereafter, the resultant steel sheet is coated with an insulating coating solution and subjected to heat flattening. In this case, a seam or spotty flaw, recess or groove is imparted to the surface of the steel sheet by a laser beam, a sprocket roll, a press, marking, local etching or the like before or after the heat flattening.

The conditions of the flaw, recess, or groove vary depending upon the usage of electrical steel sheets. When customers use the electrical steel sheet without effecting stress relieving annealing in the fabrication of iron cores, the depth may be as small as less than 5 µm for the purpose of utilizing the effect attained by a suitable strain. On the other hand, when the electrical steel sheet is used for the fabrication of a coil-wound core which requires stress relieving annealing, the flaw, recess or groove conditions are important. In this case, the flaw, recess or groove is imparted in a depth of 5 to 50 µm at intervals of 2 to 15 mm and an angle of 45 to 90° to the rolling direction. The angle is preferably as close to 90° as possible. When an decrease in the angle is required for reasons of workability, the effect of provision of the flaw, recess or groove can be attained when the angle is 45° or more. Although the width of the flaw, recess or groove is not particularly limited, it is preferably as narrow as possible. When the depth is less than 5 µm, the effect of improving the iron loss value after annealing is small. On the other hand, when the depth exceeds 50 µm, the lowering in the magnetic flux density becomes large, which is disadvantageous from the viewpoint of properties at a high magnetic field. When the direction of the seam flaw is outside the above-described range, the effect of improving the iron loss cannot be attained, or there occurs a deterioration in the iron loss.

Then, an inorganic, organic or semi-organic coating solution agent or the like is used as an insulating coating solution forming agent for coating and baking depending upon the purpose of use of the electrical steel sheet. When the tension effect and heat resistance are required, the steel sheet is subjected to coating and baking with a treating agent composed mainly of colloidal silica and a phosphate or a treating agent consisting of a phosphate alone. The coating thickness is limited to 2 to 6 µm. When the thickness is smaller than this range, no effect is attained. On the other hand, when the thickness exceeds this range, the lowering in the space factor causes properties to be lost when the product is incorporated into a transformer. When a good workability is required, the steel sheet is subjected to coating and baking with an inorganic, organic or semi-organic coating solution agent once or twice or more.

It is considered through the following mechanism that a material having an ultra low iron loss free from a glass film can be obtained by the present invention.

In the present invention, at the outset, a suitable amount of a glass film is formed in the first half of the step of the temperature rise in the final box annealing through the utilization of a suitable amount of an oxide film having a regulated reactivity formed in the decarburization annealing, MgO having a regulated reactivity and additives. This imparts a suitable sealing effect to the surface of the steel sheet, which contributes to stabilization of inhibitors such as AlN. Then, in the second half of the temperature rise in the final box annealing, etching and decomposition reaction of the glass film proceeds by virtue of the action of additives incorporated into MgO, such as chlorides, carbonates, sulfates, nitrates and sulfides. Further, in subsequent soaking at a high temperature in the final box annealing, a thermal etching effect occurs. In this stage, uneven portions of the surface of the matrix of the steel sheet caused by surface roughening during cold rolling, formation of an uneven oxide film in the decarburization annealing, etc. are smooth, so that the surface of the steel sheet becomes specular. This is because the movement of atoms on the surface during heat treatment at a high temperature is facilitated by rendering the surface of the steel sheet glassless, which lowers the surface tension, so that the surface of the steel sheet is smooth. In such a reaction process, the stabilization and strengthening of the inhibitor are important until the secondary recrystallization begins. For this reason, in the present invention, the N₂ partial pressure is controlled. This enables the stabilization of the inhibitor to be maintained, so that a grain oriented electrical steel sheet having a high magnetic flux density can be provided.

When the glassless grain oriented electrical steel sheet having a high magnetic flux density thus obtained is subjected to division of magnetic domain, a significant improvement in the iron loss can be attained over the iron loss of the conventional grain oriented electrical steel sheet having a glass film and a high magnetic flux density.

This effect is believed to reside in the following fact. Two effects, i.e., an effect derived from the freedom from a glass film and an internal oxide layer observed in products having a glass film and an effect refinning from the smooth surface having a low unevenness, prevent the occurrence of a pinning phenomenon in the movement of the domain wall during division of the magnetic domain. This combines with the effect of a high magnetic flux density to provide a significant effect, so that a material having an ultra low iron loss can be provided.

### EXAMPLES

The function and effect of the present invention will now be descried with reference to the following Examples.

### Example 1

A steel comprising, in terms of by weight, 3.50% of Si, 0.054% of C, 0.14% of Mn, 0.008% of S, 0.0295% of Al and 0.073% of N with the balance consisting of Fe and unavoidable impurities was cast into a slab by continuous casting. The slab was heated to 1,200°C, hot-rolled, annealed, pickled and cold-rolled into a sheet having a thickness of 0.22 mm which was then subjected to decarburization annealing for 110 sec. In this case, the decarburization annealing was effected on the two temperature levels of 830°C and 840°C. The average grain diameter of the primary recrystallized grains and the proportion of grains having a diameter more than twice as large as the average grain diameter are shown in Fig. 2. The steel sheets subjected to decarburization annealing were nitrided to have a nitrogen (N) content of 226 ppm, coated with an annealing separator comprising a chloride, a carbonate, a nitrate, a sulfate or the like and then subjected to final box annealing. The high temperature final box annealing cycle was effected under two conditions shown in Figs. 1 (A) and 1 (B). In a continuous line, the steel sheets subjected to secondary recrystallization was mildly pickled with 2.5% sulfuric acid solution at 80°C for 10 sec, coated with an insulating coating solution agent comprising 50 kg of 50% Al(H₂PO₄)₃, 70 kg of 30% colloidal silica and 5 kg of CrO₃, and then subjected to baking and heat flattening at 850°C for 30 sec. Thereafter, a strain was imparted to the steel sheets in the perpendicular direction to the rolling direction under conditions of intervals of 5 mm in the rolling direction, an irradiation width of 0.15 mm and an irradiation mark depth of 2.0 µm to provide final products.

Conditions for additive to annealing separators are listed in Table 1, and the test results are given in Table 2.

**Table 1**

| No. | Annealing Separator Conditions |
|---|---|
| 1 Invention | MgO 100 g + CaCl₂ 5 g |
| 2 Do. | Do. + SnCl₂ 7 g |
| 3 * | Do. + Al₂(SO₄)₃ 3 g |
| 4 Do. | Do. + SrCl₂ 5 g + MgCl₂ 5 g |
| 5 * | Do. + FeS 7 g + K₂CO₃ 8 g |
| 6 Comp. Ex. | Do. + CaCl₂ 0.5 g + K₂CO₃ 0.5 g |
| 7 * | Do. + TiO₂ 5 g + Na₂B₄O₇ 0.2 g |

| | |
|---|---|
| * Examples not forming part of the invention | |

**Table 2**

| Magnetic Properties of Product Sheet: B₈ value (T)/W_{17/50} value (w/kg) (―: failure of secondary recrystallization) | | | |
|---|---|---|---|
| Annealing Separator No. | Decarburization Annealing Temp. | Final box Annealing Cycle | |
| | | A | B (Comparative Material) |
| 1 | 830°C | *1.96/0.63 | 1.86/0.87 |
| | 840°C | 1.88/0.84 | ― |
| | | | |
| 2 | 830°C | *1.95/0.66 | 1.86/0.89 |
| | 840°C | 1.86/0.88 | ― |
| | | | |
| 3 | 830°C | 1.94/0.69 | 1.84/0.92 |
| | 840°C | 1.86/0.88 | ― |
| | | | |
| 4 | 830°C | *1.95/0.65 | 1.85/0.89 |
| | 840°C | 1.87/0.86 | ― |
| | | | |
| 5 | 830°C | 1.94/0.69 | 1.85/0.90 |
| | 840°C | 1.85/0.90 | ― |
| | | | |
| 6 | 830°C | *1.91/0.78 | 1.90/0.81 |
| | 840°C | 1.89/0.81 | 1.90/0.81 |
| | | | |
| 7 | 830°C | 1.92/0.78 | 1.91/0.79 |
| | 840°C | 1.90/0.83 | 1.90/0.80 |

| | | | |
|---|---|---|---|
| (*: Invention) | | | |

In all the materials of the present invention, the thickness of the oxide film on the surface of the steel sheet before coating with an insulating film was 0.3 µm or less, that is, the surface could be successfully rendered glassless. When the heating rate in the final box annealing was lowered, a very high B₈ value could be obtained by enhancing the N₂ partial pressure and lowering the decarburization annealing temperature.

### Example 2

A steel material comprising, in terms of by weight, 0.054% of C, 3.35% of Si, 0.12% of Mn, 0.032% of acid soluble Al, 0.007% of S and 0.0072% of N with the balance consisting of Fe and unavoidable impurities was hot-rolled into a sheet having a thickness of 1.6 mm, annealed at 1130°C for 2 min, pickled and cold-rolled into a sheet having a final thickness of 0.15 µm.

Then, the steel sheet was subjected to decarburization annealing under conditions of 25% N₂ + 75% H₂ and a dew point of 65°C at 830°C for 70 sec, and nitrided in a dry atmosphere comprising 25% of N₂, 75% of H₂ and NH₃ at 750°C for 30 sec to have a nitrogen (N) content of 220 ppm, thereby providing a material under test. This steel sheet was coated with an annealing separator having a composition specified in Table 3, and final box annealing was effected with the atmosphere conditions being changed to those shown in Figs. 1 (A) and 1 (B). This steel sheet was mildly pickled with 2% H₂SO₄ at 80°C for 10 sec to activate the surface of the steel sheet. The surface of the steel sheet was coated with an insulating coating solution comprising 100 ml of 20% colloidal SiO₂, 25 ml of 50% monobasic aluminum phosphate, 25 ml of 50% monobasic magnesium phosphate and 7 g of chromic anhydride so that the thickness of the film after baking was 4 µm, and subjected to baking at 830°C for 30 sec to provide a product. The surface appearance, coverage of glass film and magnetic properties of the steel sheets in this experiment are given in Table 4.

**Table 3**

| | Coating Conditions for Annealing Separator | | | |
|---|---|---|---|---|
| No. | MgO | Cl Content of Chloride | S Content of Chloride | N Content of Nitride |
| 8 Invention | CAA 60 sec 100 pt.wt. | KCl 3 pt.wt. | Cas 1 pt.wt. | MnN 2 pt.wt. |
| 9 Do. | Do. | CaCl₂ | Na₂S | Do. |
| | Do. | Do. | Do. | Do. |
| 10 Do. | Do. | FeCl₃ | CuS | Do. |
| | Do. | Do. | Do. | Do. |
| 11 Do. | Do. | MgCl₂ 1.5 + | Al₂S₃ | Do. |
| | Do. | CaCl₂ 1.5 | Do. | Do. |
| 12 Do. | Do. | MnCl₂ 1.5 + | BaS | Do. |
| | Do. | LiCl 1.5 | Do. | Do. |
| 13 Comp.Ex. | CAA 60 sec 100 pt.wt. + TiO₂ 5 pt.wt. + Na₂B₄O₇ 0.3 pt.wt. | | | |

As is apparent from the results, in all the materials coated with the annealing separators according to the present invention, the surface could be substantially completely rendered glassless and exhibited a metallic gloss, so that steel sheets having a specular surface could be provided. In all the materials according to the present invention, the coverage of glass was 1 g/m² or less, that is, the glass film was hardly formed. With respect to magnetic properties, all the materials subjected to final box annealing under conditions (A) had a high magnetic flux density and a low iron loss value, whereas all the materials subjected to final box annealing under comparative conditions (B) were poor in secondary recrystallization and had poor magnetic properties. All the materials according to the present invention were far superior to the comparative materials in the repeated flexural property. Further, with respect to the number of times of punching as well, the materials according to the present invention exhibited remarkably excellent results.

### Example 3

The same material as that used in Example 2 was subjected to the same treatment as that of Example 2 and hot-rolled into a sheet having a final thickness of 0.225 mm. This steel sheet was subjected to decarburization annealing under conditions of 25% N₂ + 75% H₂ and a dew point of 65°C at 840°C for 90 sec, and subsequently annealed in a dry atmosphere comprising 25% of N₂, 75% of H₂ and NH₃ at 750°C for 30 sec with the NH₃ content being varied to have a nitrogen (N) content of 200 ppm. Thereafter, the steel sheet was coated with an annealing separator having a composition specified in Table 5, and final box annealing was effected under conditions shown in Figs. 1 (A). The surface of the steel sheet was coated with a coating agent comprising 100 ml of 2.0% colloidal SiO₂, 50 ml of 50% Mg(H₂PO₄)₂ and 7 g of CrO₃ and subjected to baking with the film thickness being varied. The results on the state of the film and magnetic properties in this experiment are given in Table 6.

**Table 5**

| | Coating Conditions for Annealing Separator | | | |
|---|---|---|---|---|
| No. | MgO | Cl Content of Chloride | S Content of Chloride | N Content of Nitride |
| 14 Invention | CAA 75 sec 100 pt.wt. | SnCl₂ 1.5 pt.wt. | MgSO₄ 3.0 pt.wt. | Si₃N₄ 5 pt.wt. |
| 15 Do. | Do. | Do. | Na₂SO₄ | Do. |
| | | 5.0 pt.wt. | Do. | Do. |
| 16 Do. | Do.. | Do. | CuSO₄ | Do. |
| | | 10.0 pt.wt. | Do. | Do. |
| 17 Comp.Ex. | CAA 75 sec 100 pt.wt. + TiO₂ 5 pt.wt. + Na₂B₄O₇ 0.3 pt.wt. | | | |

As is apparent from the results, in all the materials according to the present invention, the surface could be significantly rendered glassless and exhibited a metallic gloss, and the coverage of the formed glass film was 1 g/m² or less. With respect to magnetic properties as well, all the materials coated with the annealing separator according to the present invention had good iron loss and magnetic flux density values. A particularly good iron loss value could be obtained when the film thickness was 3 µm or more. Also in the N and S contents of the steel, the glassless materials according to the present invention exhibited a significantly lower value than the comparative material having a glass film.

The comparative material having a glass film was unsuccessful in the purification and had a poor iron loss value.

### Example 4

A steel material comprising, in terms of by weight, 0.054% of C, 3.35% of Si, 0.10% of Mn, 0.030% of acid soluble Al, 0.007% of S and 0.007% of N with the balance consisting of Fe and unavoidable impurities was hot-rolled into a sheet having a thickness of 2.0 mm, annealed at 1130°C for 2 min, pickled and cold-rolled into a sheet having a final thickness of 0.225 mm.

Then, the steel sheet was subjected to decarburization annealing under conditions of 25% N₂ + 75% H₂ and a dew point of 55°C at 830°C for 100 sec, and nitrided in a dry atmosphere comprising 25% of N₂, 75% of H₂ and NH₃ at 750°C for 30 sec to have a nitrogen (N) content of 250 ppm to provide a material under test.

This steel sheet was coated with an annealing separator having a composition specified in Table 7, and final box annealing was effected with the atmosphere conditions being changed to those shown in Figs. 1 (A) and 1 (C). This steel sheet was mildly pickled with 2% H₂SO₄ at 80°C for 10 sec to activate the surface of the steel sheet. The surface of the steel sheet was coated with an insulating coating solution agent comprising 80 ml of 20% colloidal SiO₂, 20 ml of 20% colloidal ZrO₂, 50 ml of 50% Al(H₂PO₄)₃ and 7 g of CrO₃ so that the thickness of the film after baking was 4 µm, and subjected to baking at 830°C for 30 sec to provide a product. The surface appearance, coverage of glass film and magnetic properties of steel sheets in this experiment are given in Table 7.

**Table 7**

| No. | Coating Conditions for Annealing Separator |
|---|---|
| 18 Invention | MgO 100 pt.wt. + FeCl₃ 10 pt.wt. |
| | |
| 19 Do. | MgO 100 pt.wt. + CaCl₂ 5 pt.wt. + CaS 5 pt.wt. |
| | |
| 20 Do. | MgO 100 pt.wt. + BaCl₂ 5 pt.wt. + KCl 5 pt.wt. |
| | |
| 21 Do. | MgO 100 pt.wt. + SnCl₂ 5 pt.wt. + ZnCl₂ 5 pt.wt. + MgS 5 pt.wt |
| | |
| 22 Do. | MgO 100 pt.wt. + NaCl 10 pt.wt. + FeS 10 pt.wt. |
| 23 Comp.Ex. | MgO 100 pt.wt. + TiO₂ 5 pt.wt. + Na₂B₄O₇ 0.3 pt.wt. |

As is apparent from the results, in all the materials according to the present invention, the surface could be substantially rendered completely glassless, and a good glassless uniform surface appearance could be obtained. With respect to magnetic properties, all the materials subjected to finish annealing under conditions (A) had a high magnetic flux density and a lower iron loss value than the comparative material having a glass film, whereas all the materials subjected to final box annealing under conditions (C) had an extremely low magnetic flux density and were a poor material. All the materials according to the present invention were far superior in the surface roughness to the materials having a glass film, that is, it was confirmed that the surface appearance was improved by the present invention. Further, the materials according to the present invention exhibited a great improvement in the punchability as a measure for the evaluation of workability.

### Example 5

The same material as that used in Example 4 was subjected to the same treatment as that of Example 4 and rolled into a sheet having a final thickness of 0.225 mm. A seam flaw was imparted to the steel sheet by using a laser beam in the rolling direction and a direction normal to the rolling direction of the steel sheet under conditions of an interval of 5 mm, a depth of 5 µm and a width of 100 µm, and the steel sheet was then subjected to decarburization annealing under conditions of 25% N₂ + 75% H₂ at 830°C for 100 sec and nitrided in an atmosphere comprising 25% of N₂, 75% of H₂ and NH₃ to have a nitrogen (N) content of 220 ppm. Thereafter, the steel sheet was coated with an annealing separator having a composition specified in Table 9, and final box annealing was effected under conditions shown in Fig. 1 (A). The surface of the steel sheet was coated with an insulating film forming agent comprising 70 cc of 20% colloidal SiO₂, 25 cc of 20% colloidal ZrO₂, 5 cc of 20% colloidal SnO₂, 50 cc of 50% monobasic magnesium phosphate and 5 g of CrO₃ and subjected to baking with the coating thickness being varied. The results on the state of the film and magnetic properties in this experiment are given in Table 10.

**Table 9**

| No. | Coating Conditions for Annealing Separator |
|---|---|
| 24 Invention | MgO 100 pt.wt. + MnCl₂ 10 pt.wt. + SnCl₂ 5 pt.wt. |
| | |
| 25 Invention | MgO 100 pt.wt. + CaCl₂ 5 pt.wt. + MgCl₂ 5 pt.wt. + SrS 5 pt.wt. |
| 26 Comp.Ex. | MgO 100 pt.wt. + TiO₂ 5 pt.wt. + Na₂B₄O₇ 0.3 pt.wt. |

As is apparent from the results, in all the materials according to the present invention, the surface could be substantially completely rendered glassless and exhibited a metallic gloss. On the other hand, in the material coated with a comparative annealing separator, a uniform glass film was formed as with Example 4. With respect to magnetic properties as well, all the materials subjected according to the present invention had a good iron loss value, and a particularly good iron loss value was obtained when the coverage of the insulating film was 3 to 4.5 µm. By contrast, in the comparative material, the attained iron loss values were inferior to those in the materials according to the present invention.

As is apparent from the above-described Examples, according to the present invention, grain oriented electrical steel sheets not having a glass film and having a very high magnetic flux density and an ultra low iron loss, particularly grain oriented electrical steel sheets having a high magnetic flux density and a low iron loss and significantly excellent in the workability, such as slittability, cuttability and punchability, can be produced at a low cost.

## Claims

1. A process for producing a grain oriented electrical steel sheet having a high magnetic flux density and an excellent iron loss property by heating a slab at a low temperature, said process comprising the step of: heating a slab comprising, in terms of by weight, 0.021 to 0.075% of C, 2.5 to 4.5% of Si, 0.010 to 0.040% of acid soluble Al, 0.0030 to 0.0130% of N, optionally 0.03 to 0.15 % of P, 0.0140% or less of S and 0.05 to 0.45% of Mn with the balance consisting of Fe and unavoidable impurities at a temperature below 1,280°C, hot-rolling the heated slab and optionally subjecting the hot-rolled sheet to annealing, subjecting the steel sheet to once or twice or more cold rolling with annealing between the cold rollings being effected to provide a steel sheet having a final thickness, subjecting the cold-rolled sheet to decarburization annealing, nitriding the steel sheet, coating the nitrided steel sheet with an annealing separator, subjecting the coated steel sheet to final box annealing and coating the annealed steel sheet with an insulating film, wherein said annealing separator comprises at least a Cl compound in an amount of 1 part by weight or more in terms of Cl based on 100 parts by weight of MgO and the heating in the final box annealing is effected in an atmosphere comprising N₂ and H₂ with the nitrogen content being 30% or more at a heating rate of 20°C/hr or less.

2. The process for producing a grain oriented electrical steel sheet having a high magnetic flux density and an excellent iron loss property according to claim 1, wherein said annealing separator contains as an additive at least one member selected from the group consisting of Cl compounds, S compounds, carbonates, nitrates and sulfates in an amount of 1 to 15 parts by weight in terms of the total amount of Cl, S, (CO₃)⁻² and (SO₄)⁻².

3. The process for producing a grain oriented electrical steel sheet having a high magnetic flux density and an excellent iron loss property according to claim 1, wherein the amount of oxygen added to the steel sheet in the decarburization annealing is 900 ppm or less and the Fe-oxide to SiO₂ ratio in the oxide film is 0.20 or less.

4. The process for producing a grain oriented electrical steel sheet having a high magnetic flux density and an excellent iron loss property according to claim 1, wherein the amount of nitrogen added to the steel sheet in the nitriding treatment process is 150 ppm or more.

5. The process for producing a grain oriented electrical steel sheer having a high magnetic flux density and an excellent iron loss property according to claim 1 or 2, wherein said annealing separator comprises 100 parts by weight of MgO and, added thereto, 2 to 30 parts by weight of at least one member selected from the group consisting of chlorides, carbonates, nitrates, sulfates and sulfides of Li, K, Bi, Na, Ba, Ca, Mg, Zn, Fe, Zr, Sn, Sr, Al, etc., the MgO used in the annealing separator having such a particle size that 30% or more of the MgO consists of particles having a diameter of 10 µm or less, a citric acid activity (CAA value) of 50 to 300 sec (as measured at 30°C) and a hydration ig-loss of 5% or less.

6. The process for producing a grain oriented electrical steel sheet having a high magnetic flux density and an excellent iron loss property according to claims 1, wherein, in the coating of the steel sheet with the insulating film, a baking treatment is effected once or twice or more so that the film thickness after baking is in the range of from 2 to 6 µm.

7. The process for producing a grain oriented electrical steel sheet having a high magnetic flux density and an excellent iron loss property according to claim 1, wherein a seam or spotty recess or strain is imparted at an angle of 45 to 90° to the rolling direction of the steel sheet at intervals of 2 to 15 mm, a recess depth of 1 to 25 µm and a recess width of 500 µm or less by a press, a sprocket roll, marking, a laser beam, local etching, etc. after at least one step of cold rolling, decarburization annealing, finish annealing and insulating film treatment to effect the division of magnetic domain.

## Patentansprüche

1. Verfahren zur Herstellung von kornorientiertem Elektrostahlblech mit hoher magnetischer Flussdichte und ausgezeichneten Eisenverlusteigenschaften durch Erhitzen einer Bramme auf eine niedrige Temperatur,
wobei das Verfahren die Schritte umfasst:
Erhitzen einer Bramme, umfassend in Gewichtsprozent 0,021 bis 0,075% C, 2,5 bis 4,5% Si, 0,010 bis 0,040% säurelösliches Al, 0,0030 bis 0,0130% N, gegebenenfalls 0,03 bis 0,15% P, 0,0140% oder weniger S und 0,05 bis 0,45% Mn, wobei der Rest aus Fe und unvermeidbaren Verunreinigungen besteht, auf eine Temperatur unterhalb von 1.280 °C, Warmwalzen der erhitzten Bramme und gegebenenfalls Glühen des warmgewalzten Blechs, ein- oder zweimaliges oder öfteres Kaltwalzen des Stahlblechs, wobei zwischen den Kaltwalzungen geglüht wird, um ein Stahlblech mit einer Enddicke bereitzustellen, Decarbonisierungsglühen des kaltgewalzten Blechs, Nitrieren des Stahlblechs, Beschichten des nitrierten Stahlblechs mit einem Glühseparator, Endkistenglühen des beschichteten Stahlblechs und Beschichten des geglühten Stahlblechs mit einem Isolierfilm, wobei der Glühseparator wenigstens eine Cl-Verbindung in einer Menge von 1 Gewichtsteil oder mehr, ausgedrückt als Cl, bezogen auf 100 Gewichtsteile MgO umfasst, und das Erhitzen beim Endkistenglühen in einer Atmosphäre, umfassend N₂ und H₂ mit einem Stickstoffgehalt von 30% oder mehr, mit einer Aufheizgeschwindigkeit von 20 °C/h oder weniger erfolgt.

2. Verfahren zur Herstellung von kornorientiertem Elektrostahlblech mit hoher magnetischer Flussdichte und ausgezeichneten Eisenverlusteigenschaften nach Anspruch 1, wobei der Glühseparator als Zusatzstoff wenigstens einen Vertreter, ausgewählt aus Cl-Verbindungen, S-Verbindungen, Carbonaten, Nitraten und Sulfaten, in einer Menge von 1 bis 15 Gewichtsteilen enthält, bezogen auf die Gesamtmenge an Cl, S, (CO₃)²⁻ und (SO₄)²⁻.

3. Verfahren zur Herstellung von kornorientiertem Elektrostahlblech mit hoher magnetischer Flussdichte und ausgezeichneten Eisenverlusteigenschaften nach Anspruch 1, wobei die Menge an Sauerstoff, die dem Stahlblech beim Decarbonisierungsglühen zugegeben wird, 900 ppm oder weniger beträgt und das Verhältnis von Fe-Oxiden zu SiO₂ im Oxidfilm 0,20 oder weniger beträgt.

4. Verfahren zur Herstellung von kornorientiertem Elektrostahlblech mit hoher magnetischer Flussdichte und ausgezeichneten Eisenverlusteigenschaften nach Anspruch 1, wobei die Menge an Stickstoff, die dem Stahlblech beim Nitrierverfahren zugegeben wird, 150 ppm oder mehr beträgt.

5. Verfahren zur Herstellung von kornorientiertem Elektrostahlblech mit hoher magnetischer Flussdichte und ausgezeichneten Eisenverlusteigenschaften nach Anspruch 1 oder 2, wobei der Glühseparator 100 Gewichtsteile MgO und, dazu zugegeben, 2 bis 30 Gewichtsteile wenigstens eines Vertreters, ausgewählt aus Carbonaten, Nitraten, Sulfaten und Sulfiden von Li, K, Bi, Na, Ba, Ca, Mg, Zn, Fe, Zr, Sn, Sr, Al usw., umfasst, wobei das im Glühseparator eingesetzte MgO eine solche Teilchengröße aufweist, dass 30% oder mehr des MgO aus Teilchen mit einem Durchmesser von 10 µm oder weniger, einer Zitronensäureaktivität (CAA-Wert) von 50 bis 300 s (gemessen bei 30 °C) und einem Hydratations-ig-Verlust von 5% oder weniger bestehen.

6. Verfahren zur Herstellung von kornorientiertem Elektrostahlblech mit hoher magnetischer Flussdichte und ausgezeichneten Eisenverlusteigenschaften nach Anspruch 1, wobei bei der Beschichtung des Stahlblechs mit dem Isolierfilm ein- oder zweimal oder öfter ein Einbrennen durchgeführt wird, so dass die Filmdicke nach dem Einbrennen im Bereich von 2 bis 6 µm liegt.

7. Verfahren zur Herstellung von kornorientiertem Elektrostahlblech mit hoher magnetischer Flussdichte und ausgezeichneten Eisenverlusteigenschaften nach Anspruch 1, wobei eine Furche oder gepunktete Vertiefung oder Verspannung unter einem Winkel von 45 bis 90° zur Walzrichtung des Stahlblechs mit Abständen von 2 bis 15 mm, einer Vertiefungstiefe von 1 bis 25 µm und einer Vertiefungsbreite von 500 µm oder weniger mittels einer Presse, einer Zahnwalze, Anreißen, Laserstrahl, lokalem Ätzen usw. nach wenigstens einem Schritt des Kaltwalzens, Decarbonisierungsglühens, Schlussglühens und der Isolierfilmbehandlung aufgebracht wird, um die Aufteilung der magnetischen Domänen zu bewirken.

## Revendications

1. Procédé de production de tôle électrique à grain orienté, ayant une densité élevée de flux magnétique et une excellente propriété de pertes dans le fer, par chauffage d'une brame à basse température, le procédé comprenant l'étape de chauffage d'une brame qui contient, en poids, 0,021 à 0,075 % de C, 2,5 à 4,5 % de Si, 0,010 à 0,040 % de Al soluble dans l'acide, 0,0030 à 0,0130 % de N, éventuellement 0,03 à 0,15 % de P, au plus 0,0140 % de S et 0,05 à 0,45 % de Mn, le reste étant constitué de Fe et des impuretés inévitables, à une température inférieure à 1 280 °C, de laminage à chaud de la brame chauffée et éventuellement de recuit de la tôle laminée à chaud, d'exécution sur la tôle, une fois, deux fois ou plus, d'un laminage à froid avec recuit entre les laminages à froid pour la formation d'une tôle ayant une épaisseur finale, de recuit de décarburation de la tôle laminée à froid, de nitruration de la tôle, de revêtement de la tôle nitrurée par un séparateur de recuit, de recuit final en caisse de la tôle revêtue, et de revêtement de la tôle recuite d'un film isolant, dans lequel le séparateur de recuit contient au moins un composé de Cl en quantité au moins égale à une partie en poids sous forme de Cl par rapport à 100 parties en poids de MgO, et le chauffage du recuit final en caisse est réalisé en atmosphère contenant N₂ et H₂, la teneur en azote étant supérieure ou égale à 30 %, avec une vitesse de chauffage inférieure ou égale à 20 °C/h.

2. Procédé de production de tôle électrique à grain orienté, ayant une densité élevée de flux magnétique et une excellente propriété de pertes dans le fer selon la revendication 1, dans lequel le séparateur de recuit contient, comme adjuvant, le composé de Cl et éventuellement au moins un composé choisi parmi les composés de S, les carbonates, les nitrates et les sulfates en quantité de 1 à 15 parties en poids, exprimée par la quantité totale de Cl, S, (CO₃)⁻² et (SO₄)⁻².

3. Procédé de production de tôle électrique à grain orienté, ayant une densité élevée de flux magnétique et une excellente propriété de pertes dans le fer selon la revendication 1, dans lequel la quantité d'oxygène ajoutée à la tôle pendant le recuit de décarburation est inférieure ou égale à 900 ppm et le rapport de l'oxyde de Fe à SiO₂ dans le film d'oxyde est inférieur ou égal à 0,20.

4. Procédé de production de tôle électrique à grain orienté, ayant une densité élevée de flux magnétique et une excellente propriété de pertes dans le fer selon la revendication 1, dans lequel la quantité d'azote ajoutée à la tôle dans l'opération de traitement par nitruration est supérieure ou égaie à 150 ppm.

5. Procédé de production de tôle électrique à grain orienté, ayant une densité élevée de flux magnétique et une excellente propriété de pertes dans le fer selon la revendication 1 ou 2, dans lequel le séparateur de recuit contient 100 parties en poids de MgO et, sous forme ajoutée, 2 à 30 parties en poids d'au moins un composé choisi dans le groupe constitué par les carbonates, les nitrates, les sulfates et les sulfures de Li, K, Bi, Na, Ba, Ca, Mg, Zn, Fe, Zr, Sn, Sr, Al, etc., MgO utilisé dans le séparateur de recuit ayant une dimension particulaire telle que 30 % au moins de MgO sont constitués de particules ayant un diamètre inférieur ou égal à 10 µm, une activité à l'acide citrique (valeur CAA) de 50 à 300 s (mesurée à 30 °C), et une perte au feu d'hydratation inférieure ou égale à 5 %.

6. Procédé de production de tôle électrique à grain orienté, ayant une densité élevée de flux magnétique et une excellente propriété de pertes dans le fer selon la revendication 1, dans lequel, dans le revêtement de la tôle par le film isolant, un traitement de cuisson est réalisé une fois, deux fois ou plus afin que l'épaisseur du film après cuisson soit comprise entre 2 et 6 µm.

7. Procédé de production de tôle électrique à grain orienté, ayant une densité élevée de flux magnétique et une excellente propriété de pertes dans le fer selon la revendication 1, dans lequel une cavité ou déformation de forme allongée ou localisée est appliquée avec un angle de 45 à 90° par rapport à la direction de laminage de la tôle à des intervalles de 2 à 15 mm, une profondeur de cavité de 1 à 25 µm et une largeur de cavité inférieure ou égale à 500 µm, par une presse, un cylindre conformé, un marquage, un faisceau laser, une attaque locale, etc., après au moins une étape de laminage à froid, un recuit de décarburation, un recuit de finition et un traitement par un film isolant pour assurer la division du domaine magnétique.
